

## UNITED STATES PATENT OFFICE

2,669,543

## LUBRICANT

Sabine Hirsch, Minneapolis, Minn., assignor to  
 Cargill, Incorporated, Minneapolis, Minn., a  
 corporation of Delaware

No Drawing. Application April 15, 1949,  
 Serial No. 87,839

12 Claims. (Cl. 252—35)

**1** This invention relates to lubricants and to processes of preparing them. It refers to lubricants consisting of a mineral oil and a soap which has been made from oxidized hydrocarbons. Moreover, the invention refers to lubricants in which the soap is made from oxidized hydrocarbons which are compatible with vegetable or animal fats, or fatty acids, so that mixtures of them could be used for lubricants which are intended to have special properties.

Heretofore, it has been the general practice to utilize natural fats or fatty acids, or mixtures thereof, of animal or vegetable origin in making soaps for greases. The better quality greases are made from refined or hydrogenated fats or fatty acids, but the bulk of the grease is made from low-grade animal fats which have a bad odor and a high percentage of rancidity. Sometimes the odor can be masked by cheap perfume, but this will disappear in time and leave the objectionable odor in the grease, when the same is stored for a longer time. Furthermore, these low-grade fats are not always uniform in quality, and therefore, the grease maker is never certain of being able to produce greases of uniform quality. But even when refined fats or fatty acids are used, it is the general practice to add anti-oxidants to prevent rancidity and oxidation.

In the present invention where oxidized hydrocarbons are used for the soap base, the greases made of this product are always of uniform quality because the oxidation by which these hydrocarbons are obtained can be directed always in the same way. Any saponification number desired can be obtained. These oxidized hydrocarbons never get rancid or obtain an objectionable odor so that lubricants made from soap base using them do not need the addition of anti-oxidants.

A particular feature of the present invention is the fact that lubricants can be made from oxidized hydrocarbons, as such, without the addition of any animal or vegetable fats or fatty acids. The lubricants so obtained have very great stability, a low break-down when worked, and a very good oiliness, that means they have the property to wet metal surfaces well and leave on the metal a film which is not readily removed. Soap bases made from this type of oxidized hydrocarbons are compatible with paraffinic or naphthenic base mineral oils. Oxidized hydrocarbon mixtures are very easily saponified in water as well as in an oil media, which results in finished greases of good quality in a short time. Most greases can be kettle finished, thus avoiding the multiple steps

**2** of providing a homogeneous grease. It has been found, however, that oxidized hydrocarbons when used, as such, in the soap for grease making show much better stability and have a much smaller break-down percentage in the mechanical worker than greases made with soaps in which mixtures of natural fats and oxidized hydrocarbons have been used.

An object of the invention is to provide a lubricant composed of a soap made from oxidized hydrocarbons, as such, and a mineral oil to form a grease which has great stability.

Another object of this invention is to provide a lubricating grease composed of a major portion of mineral oil and a minor portion of soap made of oxidized hydrocarbons, as such, to form a grease which under standard break-down testing conditions has a break-down of less than 10%.

Another object of this invention is to provide a lubricant grease consisting of a major portion of mineral oil and a minor portion of soap made from a mixture of oxidized hydrocarbons and animal or vegetable fats, or fatty acids, or mixtures thereof, to form greases of special desired properties.

A further object is to provide a soap base for lubricant greases in which the oxidized hydrocarbons are saponified with more than one neutralizing agent so as to form a multiple soap base.

In carrying out this invention, a hydrocarbon or a hydrocarbon mixture, which at normal temperature and normal pressure is liquid or solid, or of high viscosity, is heated in a kettle with stirring facilities to a temperature preferably of 255° F., but not much higher than 300° F. In this heated mass is introduced a gas containing oxygen and carrying a minor percentage of moisture. To accelerate the oxidation, an oxidation catalyst is used, as well as a minor percentage of a metallic per-salt in an emulsion of water and an oleaginous material, and so forming an emulsion of the whole reaction mass during the time of the oxidation process. The method of oxidizing the hydrocarbons is fully described and claimed in my prior Patent 2,391,236, granted on December 18, 1945. When the oxidation has reached the desired saponification number the oxidized hydrocarbons are taken out from the kettle and washed and filtered. The washing of this product can be made with hot water, acidulated water, or salt water. After filtering the product is ready to be used for soaps and lubricants.

## GENERAL PROCEDURE

Into a grease kettle is charged 200 parts of 100

## 3

SUS at 100° F. refined naphthenic mineral oil. Then 100 parts of oxidized hydrocarbons are added, heat and stirring facilities are slowly put in action until both ingredients are dissolved. Then a calculated amount of saponifying agent in a saturated solution is poured into this mixture. Saponification starts immediately. The temperature is then slowly allowed to rise to about 220° F. to complete saponification. This temperature is maintained until most of the water has evaporated. When all of the water is gone the temperature is raised to about 280° F. and then to this basic grease mixture, 200 parts of pre-heated heavy naphthenic mineral oil of a viscosity of 240 SUS at 210° F. is added step by step. The temperature of 280° F. is maintained until all the heavier mineral oil is entirely incorporated in the grease. The grease is then ready to be poured into containers. This can be done at 280° F. or if desired the grease can be stirred down to a lower temperature and then poured into containers ready for use.

In order that the lubricant may have a stable consistency after a considerable amount of working, it is necessary that the hydrocarbons, which are always heavier aliphatic hydrocarbons varying in consistency from liquid to solid at normal temperatures, be substantially oxidized, and that the unsaponifiable materials remain in the mixture. The hydrocarbon used as the starting material may and will be of varying natures, but when oxidized to produce saponification numbers in the range of about 155-190, the product will have been oxidized to such an extent that when formed into soap produces lubricants of stable consistency that will withstand vigorous prolonged working without breakdown.

The break-down test referred to hereinafter is a standard test adopted by the A. S. T. M.

## EXAMPLE NO. 1

## Sodium grease

The procedure is described in the general description.

Used are:

200 parts of 100 SUS at 100° F. naphthenic mineral oil  
100 parts of oxidized hydrocarbon mixture sap.  
No. about 159  
12 parts of NaOH in 12 parts of water  
200 parts of heavy naphthenic mineral oil 240 SUS at 210° F.

This is a smooth, non-fibrous sodium grease of homogeneous texture, having good odor. There is no indication of syneresis after a long period of storage at temperatures over 90° F. Field tests on high speed bearings running over 1700 R. P. M. under full load showed very good lubrication and cool performance.

Consistency:

At 60 strokes 288 at 77° F.  
At 5000 strokes 300 at 77° F.

This is a break-down of 4%.

Dropping point by Ubbelohde method more than 450° F.

## EXAMPLE NO. 2

## Calcium grease

The procedure is described in the general description. Used are:

200 parts of 100 SUS at 100° F. naphthenic mineral oil

## 4

100 parts of oxidized hydrocarbon mixture sap.

No. about 155.

10.5 parts of Ca(OH)<sub>2</sub> in 15 parts of water.

A mixture of:

100 parts of 100 SUS at 100° F. naphthenic mineral oil  
100 parts of 240 SUS at 210° F. naphthenic mineral oil.

This is a buttery, clear, homogenous calcium grease which performs well as a chassis lubricant.

Consistency:

At 60 strokes 325 at 77° F.

At 5000 strokes 346 at 77° F.

This is a break-down of about 6%.

Dropping point by Ubbelohde method 200° F.

## EXAMPLE NO. 3

## Aluminum grease

Into the grease kettle, while stirring, a slurry is made of:

10 parts of 100 SUS at 100° F. naphthenic mineral oil

7.5 parts of aluminum soap made from a mixture of 50 parts of oxidized hydrocarbons and 50 parts of high molecular animal fatty acids, said fat mixture having a sap. No. of about 192.

Heat is slowly applied until a firm gelatinous soap base results. Then

107.5 parts of preheated, heavy naphthenic mineral oil, viscosity 100 SUS at 210° F. is slowly added and the temperature step by step raised to about 330° F. This temperature is kept until all the heavy oil is incorporated in the grease. The grease can now be poured into containers and after a period of about 48 hours is ready for use.

This is a smooth, clear aluminum grease, easy to handle in lubrication equipment. Field tests on chassis, slow moving bearings, and as a pressure gun lubricant, show satisfactory performance.

Consistency at 60 strokes 330 at 77° F.  
Dropping point by Ubbelohde method about 200° F.

## EXAMPLE NO. 4

## Lithium grease

Into the grease kettle we charge:

2 parts of 100 SUS at 100° F. naphthenic mineral oil and

2 parts of oxidized hydrocarbons, having a saponification number of 183. Heat is slowly applied while stirring until the oxidized hydrocarbons dissolve in the mineral oil. To this is added a hot aqueous solution of the required amount of lithium hydrate for complete saponification. The mass is brought to a temperature of about 220° F. and allowed to saponify. When most of the water evaporates the temperature is slowly increased to about 380° F. At this temperature is added:

6 parts of preheated 100 SUS at 100° F. naphthenic mineral oil. When the mass is completely homogenous the grease may be poured into containers at this temperature, or may be stirred down to a lower temperature and poured. In either case the grease is kettle finished and can be used as such.

The consistency of this grease at 60 strokes is 287 at 77° F. and at 10,000 strokes is 286 at 77° F.

So we have a smooth, light colored, uniform

grease showing a break-down of 0% at 10,000 strokes. There is no sign of syneresis when stored at about 90° F. for a period of 9 months.

The dropping point of this grease by the Ubbelohde method is 375° F.

My invention is defined in the terms of the appended claims.

I claim:

1. A lubricant, comprising mineral oil, and a soap mixture formed by reacting a saponifying agent with the product, as such, resulting from the oxidation of heavier aliphatic hydrocarbons varying in consistency from liquid to solid at normal temperature and which have been oxidized to produce a saponification number of at least 155, and forming with the mineral oil a solid to semi-solid grease of a substantially stable consistency.

2. A lubricant, comprising a major portion of mineral oil, and a minor portion of a soap mixture formed by reacting a saponifying agent with the product, as such, resulting from the oxidation of heavier aliphatic hydrocarbons varying in consistency from liquid to solid at normal temperature and which have been oxidized to produce a saponification number of at least 155, and with the mineral oil forming a solid to semi-solid grease of substantially stable consistency.

3. A lubricant, comprising a major portion of mineral oil, and a minor portion of a soap mixture formed by reacting a basic metal derivative with mixed products, as such, resulting from the liquid phase oxidation of heavier aliphatic hydrocarbons varying in consistency from liquid to solid at normal temperatures and which have been oxidized to the extent that the mixed products have a combined saponification number of at least 155 and forming with the mineral oil a solid to semi-solid grease of substantially stable consistency.

4. A lubricant, comprising a major portion of mineral oil, and a minor portion of a soap mixture formed by reacting a saponifying agent with a mixture of significant proportions of glycerides with the product, as such, resulting from the liquid phase oxidation of heavier aliphatic hydrocarbons varying in consistency from liquid to solid at normal temperatures and which have been oxidized to produce a saponification number of at least 155, the proportions of glycerides to oxidized product being related to the titer of the glycerides such that the titer of the mixture forms with the mineral oil a solid to semi-solid grease of substantially stable consistency.

5. A lubricant, comprising a major portion of mineral oil, and a soap mixture formed by reacting a saponifying agent with a mixture of sig-

nificant proportions of fatty acids derived from natural glycerides and the product, as such, resulting from the liquid phase oxidation of heavier aliphatic hydrocarbons varying in consistency from liquid to solid at normal temperatures and which have been oxidized to the extent of producing a saponification number of at least 155, the proportion of fatty acids to oxidized product being related to the titer of the fatty acids such that the titer of the mixture forms with the mineral oil a solid to semi-solid grease of substantially stable consistency.

15 6. A lubricant, comprising substantially 80% of mineral oil, and a soap mixture formed by reacting a saponifying agent with the product as such resulting from the liquid phase oxidation of heavier aliphatic hydrocarbons varying in consistency from liquid to solid at normal temperatures and which have been oxidized to produce a saponification number of at least 155, and which forms with the mineral oil a semi-solid grease of substantially stable consistency.

20 7. A lubricant as described in claim 6 in which the saponifying agent consists of an alkali metal compound.

25 8. A lubricant as described in claim 6 in which the saponifying agent consists of an alkaline earth metal compound.

30 9. A lubricant as described in claim 6 in which the saponifying agent consists of a basic metal compound of the group consisting of lithium and sodium.

35 10. A lubricant as described in claim 6 in which the saponifying agent consists of a basic metal compound of the group consisting of barium, calcium, strontium, magnesium and zinc.

35 11. A lubricant as described in claim 6 in which the saponifying agent consists of a basic metal compound of aluminum.

40 12. A lubricant as described in claim 6 in which the saponifying agent consists of a basic metal compound of lead.

SABINE HIRSCH.

References Cited in the file of this patent

UNITED STATES PATENTS

| Number    | Name                 | Date           |
|-----------|----------------------|----------------|
| 1,700,056 | James -----          | Jan. 22, 1929  |
| 2,012,252 | Burwell -----        | Aug. 20, 1935  |
| 2,055,043 | Nelson -----         | Sept. 22, 1936 |
| 2,058,237 | Kaufman et al. ----- | Oct. 20, 1936  |
| 2,137,494 | Jolly -----          | Nov. 22, 1938  |
| 2,258,300 | Morway -----         | Oct. 7, 1941   |
| 2,303,256 | Camelford -----      | Nov. 24, 1942  |
| 2,391,019 | Hirsch -----         | Dec. 18, 1945  |
| 2,391,236 | Hirsch -----         | Dec. 18, 1945  |